

[54] PROCESS FOR REACTING SULTONES  
WITH CELLULOSIC MATERIALS TO  
PRODUCE CELLULOSIC MATERIALS  
HAVING BOTH BASIC AND ACIDIC  
GROUPS AND PRODUCT PRODUCED

[75] Inventors: Truman W. Ward; Ruth R.  
Benerito, both of New Orleans;  
Ralph J. Berni; Donald M. Soignet,  
both of Metairie, all of La.

[73] Assignee: The United States of America as  
represented by the Secretary of  
Agriculture, Washington, D.C.

[22] Filed: Nov. 15, 1972

[21] Appl. No.: 306,771

[52] U.S. Cl. .... 8/116 R, 8/181

[51] Int. Cl. .... D06m 1/00

[58] Field of Search .... 8/116 R, 181

[56] References Cited

UNITED STATES PATENTS

3,506,390 4/1970 Naps ..... 8/116 R  
3,698,857 10/1972 Vigo et al. ..... 8/116 R

Primary Examiner—Stephen J. Lechert, Jr.

[57] ABSTRACT

Cellulosic material is reacted with either 2-chloroethyl diethylamine hydrochloride or 2-aminoethylsulfuric acid so that either diethylaminoethyl cellulose or aminated cellulose is formed. These materials are then reacted with a hydrocarbon sultone such as propane sultone in a suitable solvent without catalyst to add the sultone at the nitrogen group. The resultant products have both acidic and basic groups in the same molecule and are zwitterion-exchange celluloses.

6 Claims, No Drawings

**PROCESS FOR REACTING SULTONES WITH  
CELLULOSIC MATERIALS TO PRODUCE  
CELLULOSIC MATERIALS HAVING BOTH BASIC  
AND ACIDIC GROUPS AND PRODUCT PRODUCED**

A non-exclusive, irrevocable, royalty-free license in the invention herein described throughout the world for all purposes of the United States Government, with the power to grant sublicenses for such purposes, is hereby granted to the Government of the United States of America.

This invention relates to chemical modification of cellulosic derivatives. More specifically, this invention relates to the modification of diethylaminoethyl cellulose and aminated cellulose with propane sultone to yield zwitterion cellulosic derivatives which have excellent ion exchange properties. The products thus produced lend themselves to further reaction with either acid reactive or basic reactive substances.

An equation which would represent the pertinent reaction of this invention is this:



wherein R is either hydrogen or an ethyl group.

The main object of this invention is to provide a process for reacting sultones with cellulosic materials without having the need of including catalysts in the reaction bath.

Another object of this invention is to provide a process for reacting cellulosic textiles having amino groups with propane sultone to produce fibrous cellulosic derivatives having zwitterion exchange properties. Textiles thus prepared would have both acid and basic groups in the same molecule.

U.S. Pat. No. 3,506,390 discloses a process wherein aqueous sodium hydroxide has been used to produce alkali cotton which was reacted in aqueous solutions of propane sultone to produce a material containing acid sites but no basic sites and the process requires the hydroxide to be in the bath in order to effect reaction.

German Pat. No. 941,977 discloses a process by Helleberger et al. wherein certain sultones are reacted with ammonia and amines. No mention is made of reaction of the sultones with amine groups which would have the amine groups attached to cellulose.

We have now discovered that a cellulosic material with primary amine groups attached (aminized cotton) can be reacted with propane sultone to produce cellulosic materials having both basic and acidic groups. The reaction proceeds readily without need of a catalyst to yield a product with zwitterion exchange properties.

We have further discovered that cellulosic material with the related tertiary amine (DEAE) grouping can likewise be reacted with the said propane sultone. It has further been calculated that butane, pentane, and higher sultones should react in the same or similar manner.

By the process of the present invention cellulose is reacted to add an amine group to the cellulose. DEAE-cellulose can be prepared by any of several processes. An acceptable one would be that one disclosed in U.S. Pat. No. 1,777,970. Aminated cotton can best be pre-

pared by the method described in Guthrie, et al. which appears in Textile Research J. 17, pp. 625-629 (1947), with the title "Introduction of Amino Groups into Cotton Fabric by the Use of 2-Aminoethylsulfuric Acid."

5 The cellulose with the amine or DEAE group attached, for purposes of this invention, is then reacted with a hydrocarbon sultone such as the preferred sultone in solution in the proper solvent.

The preferred solvent for reacting DEAE-cellulose with the sultone is either tertiary butanol or methanol while for aminated cellulose a primary alcohol such as methanol is required. The reaction is carried out while the cellulosic material is wet with the propane sultone solution. Temperatures can be varied from 25° to 75°C, and the length of time can be varied from 1 to 24 hours. By varying the nitrogen content of the DEAE or aminated intermediate and by controlling the reaction of the sultone with the amine groups by controlling length of reaction or temperature of the reaction one can produce products with varying ratios of sulfur to nitrogen. Unreacted amine sites would increase basic character of the product.

Although cotton fabric was employed in the investigative efforts which led to this invention it is obvious that any material containing cellulosic hydroxyls can be used. This includes but is not limited to fibers, yarns, fabrics, or matrixes which contain cotton, rayon, wood, or linen. Means of bringing cellulosic material into contact with the sultone solution include immersion, dipping, padding, and spraying. Although the sultone employed throughout the investigative efforts which led to the present invention was propane sultone, it should be obvious to those skilled in the art that other sultones, such as butane sultone, can be employed in the same manner. The concentration of the sultone in the solution can be varied over a wide range although the range of 5 to 20 percent will usually suffice.

In a typical laboratory demonstration of this process a dry DEAE-cotton fabric of 0.61 meq. N per gram was immersed in a solution of 10 percent propane sultone in tertiary butanol and the immersed sample held at a temperature of 50°C for 20 hours. The sample was removed from the reactant solution and thoroughly washed with water and dried. The sample was analyzed, yielding 0.26 meq. of sulfur per gram of product. An aminated cotton of 0.55 meq. of N per gram of fabric treated the same way except for the substitution of methanol for the tertiary butanol yielded 0.39 meq. of sulfur per gram of product.

To summarize, the present invention can best be described as (1) fibrous sultone-amine cellulosics and (2) the process for producing the fibrous sultone-amine cellulosics and for imparting zwitterion-exchange properties to cotton and other cellulosic materials, the process comprising reacting the cellulosic material with a compound selected from the group consisting of 2-chloroethylidethylamine hydrochloride and 2-aminoethylsulfuric acid to form respectively the diethylaminoethyl cellulose or the aminated cellulose, which are reacted with a hydrocarbon sultone without benefit of catalyst, thereby adding the sultone to the nitrogen group.

**Example 1**

Diethylaminoethylated cotton (DEAE-cotton) was prepared from 80 × 80 weave cotton printcloth which had been desized and bleached by padding twice with

20 percent beta-chloroethyldiethylamine hydrochloride, drying at 60°C for 10 minutes, immersing in 8 percent aqueous sodium hydroxide at 95°C for 10 minutes, washing free of NaOH in dilute acetic acid, washing in tap water (pH 9) to remove the acetic acid and drying. The fabric had 0.61 meq. N/g. of fabric.

Aminized cotton was prepared from 80 × 80 weave cotton printcloth which had been desized and bleached by padding with a freshly prepared solution containing 20 percent of 2-aminoethylsulfuric acid and 30% NaOH, and curing in an oven at 120°C for 15 minutes, washing in dilute acetic acid, washing in tap water and drying. The fabric had 0.55 meq./N per gram of fabric.

Comparing DEAE and aminized cottons in methanol and tertiary butanol:

The dry DEAE cotton, aminized cotton and unmodified cotton fabrics were placed in separate cylinders containing 10 percent propane solution in either tertiary butanol or absolute methanol. The containers and contents were all held at 50°C for 20 hours before removal of the fabric samples. The fabric samples were washed thoroughly with distilled water and dried the results were as follows:

| Fabric     | Meq.N/g. | t-butanol   | Methanol    |
|------------|----------|-------------|-------------|
|            |          | Meq.S/meq.N | Meq.S/meq.N |
| Aminized   | 0.55     | 0.07        | 0.70        |
| DEAE       | 0.61     | 0.43        | 0.50        |
| Unmodified | 0        | 0           | 0           |

### EXAMPLE 2

To show that an external amine will not cause reaction with unmodified cotton:

Reactions of unmodified cotton fabric samples were tried with either ethylamine or triethylamine padded on the unmodified cotton fabric to correspond to either the primary amine of aminized cotton or the tertiary amine group of DEAE cotton. The padded samples were immersed in a 10 percent solution of propane sultone in either tertiary butanol or absolute methanol and held at 50°C for 20 hours. The fabric samples were washed thoroughly with distilled water and dried. The results were as follows:

| Fabric                           |  | % Sulfur  |          |
|----------------------------------|--|-----------|----------|
|                                  |  | t-butanol | Methanol |
| Unmodified cotton, Ethylamine    |  | 0.00      | 0.02     |
| Unmodified cotton, Triethylamine |  | 0.05      | 0.00     |

### EXAMPLE 3

To show that another alcohol such as ethanol may be substituted but a different type solvent such as DMF does not work:

Aminized cotton fabric swatches were immersed in a solution of 10 percent propane sultone in either methanol, ethanol, or DMF and held at a temperature of 50°C for 20 hours. The fabric samples were removed from the solution, washed thoroughly in distilled water and dried.

|   | Methanol |      | Ethanol | DMF  |
|---|----------|------|---------|------|
| 5 | % Sulfur | 1.26 | 1.16    | 0.10 |

### EXAMPLE 4

10 This examples shows that the amount of reaction with the propane sultone varies with the amount of nitrogen present.

DEAE cottons with different nitrogen contents were reacted with a 10 percent solution of propane sultone in tertiary butanol at 50°C for 20 hours. The samples were removed from the solution and washed with water and dried before analysis.

| 20  | % Nitrogen | % Sulfur |
|-----|------------|----------|
| 0   | .01        |          |
| 1.0 | 2.27       |          |
| 1.7 | 3.24       |          |

### EXAMPLE 5

This example shows that the concentration of propane sultone in solvent can be varied but that concentrated solutions are neither desirable nor necessary.

30 Conditions as in Example 4 except only DEAE cotton of 1.0 percent nitrogen was used and concentrations of propane sultone varied. The results were as follows:

| 35 | % Propane Sultone | % Sulfur in Product |
|----|-------------------|---------------------|
| 5  |                   | 1.07                |
| 10 |                   | 1.84                |
| 20 |                   | 1.76                |

### EXAMPLE 6

45 This example will show the effect of length of reaction on the amount of reaction.

DEAE cotton fabric samples were immersed in a 10 percent solution of propane sultone in tertiary butanol and allowed to react at 50°C for different lengths of time. After reaction the samples were removed and thoroughly washed with distilled water and dried. The results were as follows:

| 55       | 1 hr. | 3 hrs. | 6 hrs. | 16 hr. | 24 hr. | 32 hr. |
|----------|-------|--------|--------|--------|--------|--------|
| % sulfur | 1.85  | 1.90   | 2.0    | 2.25   | 2.35   | 2.45   |

### EXAMPLE 7

Example 6 except substitute aminized cotton fabric in methanol for DEAE cotton fabric in tertiary butanol. Results were as follows:

| 65       | 1 Hr. | 3 Hrs. | 6 Hrs. | 20 Hrs. |
|----------|-------|--------|--------|---------|
| % sulfur | 0.78  | 0.83   | 0.95   | 1.26    |

## EXAMPLE 8

This example will illustrate the effect of temperature on the reaction of the propane sultone with DEAE cotton.

Example 6 except use 1 hour and vary temperature. Results were as follows:

|          | 25°C | 35°C | 40°C | 50°C | 60°C | 75°C |
|----------|------|------|------|------|------|------|
| % sulfur | 1.35 | 1.60 | 1.65 | 1.85 | 2.00 | 2.25 |

## EXAMPLE 9

This example will show that a DEAE cellulose prepared commercially, sold on the open market, and existing in powder form reacts with propane sultone in the same manner as the DEAE cotton fabric prepared in our laboratory.

A DEAE anion exchange cellulose called Cellex D and sold by Bio-Rad Laboratories of Richmond, Cal. was used as the commercial product.

Conditions as in Example 1 except substitute the listed DEAE samples for the fabric samples of Example 1.

|                     | Meq. N/g. | Meq.S/meq.N |
|---------------------|-----------|-------------|
| Bio-Rad DEAE Powder | 0.72      | 0.40        |
| Our DEAE Fabric     | 0.60      | 0.43        |

30

We claim:

1. A process for imparting Zwitterion-exchange properties to diethylaminoethyl cellulose, the process comprising contacting said diethylaminoethyl cellulose with an organic solvent solution of about from 5 to 20 percent hydrocarbon sultone at 25° C. to 75° C. for about 1 to 24 hours.

2. A process for imparting Zwitterion-exchange properties to aminated cellulose, the process comprising contacting said aminated cellulose with a primary alcohol solvent solution of about from 5 to 20 percent hydrocarbon sultone at 25° C. to 75° C. for about 1 to 24 hours, using the longer periods of time with the lower temperatures.

3. The process of claim 1 wherein the hydrocarbon sultone is propane sultone.

4. The process of claim 2 wherein the hydrocarbon sultone is propane sultone.

5. The product produced by the process of claim 3 wherein the nitrogen content is as high as about 2 percent and the sulfur content is as high as about 3.5 percent with respect to the weight of the sultone-cellulose.

6. The product produced by the process of claim 4 wherein the nitrogen content is as high as about 1.0 percent and the sulfur content is as high as about 1.5 percent with respect to the weight of the sultone-cellulose.

\* \* \* \* \*

35

40

45

50

55

60

65